

(No Model.)

C. A. BROWN.

BATTERY JAR.

No. 373,334.

Patented Nov. 15, 1887.



Witnesses:

Elgin B. Merrill.  
Keney Anderson

Inventor:

Charles Alva Brown  
by S. M. Bates  
his att<sup>o</sup>.

# UNITED STATES PATENT OFFICE.

CHARLES ALVA BROWN, OF PORTLAND, MAINE.

## BATTERY-JAR.

SPECIFICATION forming part of Letters Patent No. 373,334, dated November 15, 1887.

Application filed December 29, 1886. Serial No. 222,871. (No model.)

*To all whom it may concern:*

Be it known that I, CHARLES ALVA BROWN, a citizen of the United States, residing at Portland, in the county of Cumberland and State of Maine, have invented certain new and useful Improvements in Battery-Jars; and I do declare the following to be a full, clear, and exact description of the invention, such as will enable others skilled in the art to which it appertains to make and use the same, reference being had to the accompanying drawing, and to the letters and figures of reference marked thereon, which form a part of this specification.

My invention relates to cells or jars for electric batteries; and it consists in the forming or manufacture of such a battery-jar from wood or paper pulp, said jar being impregnated with a substance—such as coal-tar—which will withstand the action of acids and the other chemicals such as are used in batteries.

Hitherto battery-jars have been made of a variety of materials—such, for instance, as glass, hard rubber, porcelain, &c.; but in all jars hitherto made the material of which they were constructed has been brittle and easily destroyed, as in the case of glass, hard rubber, and porcelain, or it has been heavy and expensive, as in the jars of various material lined with lead. Electricians have long desired a battery-jar which should have the qualities of lightness, strength, and durability, which could be readily and cheaply formed, and which should have a surface and a texture suitable to receive and retain the necessary chemical-proof treatment. Such a combination of desirable qualities is to be found in a jar constructed of pulp. It is light and, when properly formed, very strong. It readily receives and retains the necessary treatment by which it is protected from the softening action of the chemicals used in batteries.

In the drawing the figure shows half-sectional view and half elevation of one of my battery-jars.

My jar is formed from wood or paper pulp 45 on any suitable machine for the purpose. The pulp jar is then impregnated with coal-tar, the jar being immersed in the heated tar.

By the porosity of the pulp it readily receives and retains the chemical-proof liquid with 5c which it is soaked. The hot tar readily permeates the porous material and completely fills the cellular spaces. On drying, the oil of the tar oxidizes and hardens, producing increased density and toughness of the jar and rendering 55 it thoroughly proof against attack by ordinary battery-fluids.

I am aware that it has been heretofore proposed to coat the interior of wooden bottles with asphalt. Such a product is very different 60 in structure from mine, and would prove inefficient for battery purposes. The asphalt, being applied as a film to the interior of the jar, would be chilled immediately on application and could not penetrate the cellular 65 spaces. In use the rubbing action of the electrodes, in case such a vessel were used as a battery-jar, would crack the lining and cause it to scale off, exposing the naked wood to the decomposing influences of the acids. 70

I claim—

As a new article of manufacture, a battery-jar composed of pulp impregnated with coal-tar.

In testimony whereof I affix my signature in 75 presence of two witnesses.

CHARLES ALVA BROWN.

Witnesses:

ELGIN C. VERRILL,  
S. W. BATES.